

## UNITED STATES PATENT OFFICE

2,333,741

## MANUFACTURE OF CAST IRON

David B. Reeder, Evanston, Ill., assignor to Electro Metallurgical Company, a corporation of West Virginia

No Drawing. Application September 29, 1942,  
Serial No. 460,125

5 Claims. (Cl. 75—130)

The invention relates to the manufacture of cast iron.

Manganese, usually in the form of ferromanganese, is often added to molten iron during the manufacture of various types of cast irons, to produce divers beneficial effects. One of the important functions of manganese is to combine with any sulfur present in the iron and to inhibit to a large extent the adverse effects which sulfur otherwise would produce. Another reason for adding manganese to cast iron is because of its deoxidizing and general scavenging actions, which have a beneficial effect on the iron. Manganese is also added to malleable iron compositions for its retarding effect on the conversion of combined carbon to temper carbon during the malleabilizing anneal, when it is desired to produce so-called pearlitic malleable iron. Depending on various factors, from about 0.2% to about 2% of manganese may be added to cast irons for these purposes.

It has been observed that irons to which fairly large additions of manganese have been made sometimes exhibit what is known as "pinhole porosity," a condition in which minute, sometimes microscopic, subcutaneous voids or "pinholes" appear in the iron. These pinholes are quite different from the ordinary voids and imperfections caused by improper casting procedure. There is some evidence to support the hypothesis that they are caused by gases in the iron. Whatever their cause, they are objectionable and often lead to rejection of castings.

It is the chief object of this invention to inhibit the formation of pinhole porosity in cast iron to which manganese has been added.

In accordance with the invention, this object is achieved by adding to the iron, preferably concurrently with the manganese, a readily reducible metallic oxide such as iron oxide, nickel oxide, manganese oxide or chromium oxide. The most generally suitable oxide for the practice of the invention is iron oxide, and convenient sources of iron oxide are iron ores and mill scale. Preferably, the oxide used is mixed with the manganese before it is added to the iron.

The optimum quantity of metal oxide to be added to an iron in the practice of the invention is best determined empirically, being dependent on melting practice, the composition of the iron, and other factors, but in general it will be between about one-quarter of one per cent and ten per cent of the quantity of manganese added to the iron. This amount furnishes sufficient oxygen to inhibit the formation of pinholes without interfering with the beneficial effects sought by the manganese addition.

The benefits of the invention may also be attained by concurrently adding manganese and oxygen through the use of a ferromanganese

that has been partially oxidized, for example by exposure to high temperatures in an oxidizing atmosphere.

The beneficial effects obtained by the invention have been demonstrated by tests conducted under commercial conditions. They are obtainable both in the production of pearlitic malleable iron and in other cast irons. Although the invention has been described with particular reference to ferromanganese as the agent used to add manganese to molten cast iron, it is not limited to that particular addition agent, being effective with any high-manganese addition agent. Similarly, the invention is not limited to the treatment of pearlitic malleable iron but is also effective in the treatment of cast irons in general.

I claim:

1. A method of treating a molten cast iron which method comprises adding to said molten iron about 0.2% to 2% manganese and metal oxide in an amount equal to about 0.25% to 10% of the manganese addition, the oxide addition inhibiting the tendency of the manganese to form pinholes in such iron.

2. A method of treating a molten cast iron which method comprises adding to said molten iron about 0.2% to 2% manganese and iron oxide in an amount equal to about 0.25% to 10% of the manganese addition, the oxide addition inhibiting the tendency of the manganese to form pinholes in such iron.

3. In the method of producing pearlitic malleable iron which comprises adding manganese to a molten iron, the improvement which comprises adding to said iron in conjunction with said manganese addition, a quantity of metal oxide equal to about 0.25% to 10% of the amount of manganese added, to inhibit the formation of pinhole porosity in said iron.

4. In the method of producing pearlitic malleable iron which comprises adding manganese to a molten iron, the improvement which comprises adding to said iron in conjunction with said manganese addition, a quantity of iron oxide equal to about 0.25% to 10% of the amount of manganese added, to inhibit the formation of pinhole porosity in said iron.

5. In a method of treating a molten cast iron which method comprises adding to such iron a minor but substantial amount of manganese to produce desired metallurgical effects, the said addition of manganese also tending to promote the formation of undesirable pinholes in such iron, the improvement which comprises adding to such iron in admixture with the manganese a small amount of metal oxide effective to inhibit said pinhole-promoting tendency of the manganese.

DAVID B. REEDER.